

## UNITED STATES PATENT OFFICE

2,580,881

STABILIZED PETROLEUM PRODUCTS AND  
STABILIZING COMPOSITIONSCharles B. Biswell, Woodstown, N. J., assignor to  
E. I. du Pont de Nemours & Company, Wil-  
mington, Del., a corporation of DelawareNo Drawing. Application May 21, 1949,  
Serial No. 94,756

20 Claims. (Cl. 252—42.4)

1

This invention relates to petroleum products which have been stabilized against oxidation and to new compositions of matter which are particularly effective for stabilizing greases.

Petroleum products, such as gasoline, fuel oils, lubricating oils and greases tend to oxidize and deteriorate in the presence of oxygen during storage and use. It has become common practice to inhibit such oxidation and deterioration by adding to such petroleum products phenols, amines and aminophenols, commonly called antioxidants. While the use of such antioxidants has met with considerable success, the petroleum products are frequently brought into contact with copper or copper compounds, or become contaminated with copper compounds, which catalyze the oxidation and deterioration of the petroleum products and also of the antioxidants contained therein. It has, therefore, become necessary to also add to the petroleum products other materials which will overcome the catalytic effect of copper and compounds containing it, such other materials being called metal deactivators or copper deactivators.

Usually, greases are prepared by incorporating a metal soap into a petroleum oil, particularly a soap which causes the oil to gel. The most important and common soaps employed for this purpose are soaps of lithium, sodium, potassium, calcium, barium and aluminum or mixtures of such soaps. Such greases, like the petroleum oils from which they are produced, are subject to deterioration by oxidation during storage and use. Such deterioration and oxidation and the accumulation of oxidized materials in the greases greatly reduces the lubrication properties of the greases. Furthermore, this deterioration and oxidation is also catalyzed by metallic surfaces and ingredients, and particularly by copper and copper-containing metals, such as brass. This effect of copper and copper-containing metals is serious because many bearing parts are made of such metals.

It has been proposed to inhibit the deterioration and oxidation of greases by adding thereto various secondary aromatic amines, such as phenyl- $\alpha$ -naphthylamine, phenyl- $\beta$ -naphthylamine, diphenylamine and the like. As a class, such secondary aromatic amines are only moderately effective. The response is not always proportional to the concentration of the amine in the grease and it is not always possible to prepare a grease with a desired high stability to oxidation merely by increasing the concentration of the amine in the grease. Such amines are particularly ineffective in the presence of copper and copper-containing metals. Furthermore, many of such amines tend to discolor badly and impart such undesirable color to the greases, particularly when employed in high concentrations.

2

Clarkson and Pedersen, in Patent 2,353,690, disclose that 1-(ortho-hydroxy-arylidene)-aminoguanidines, represented by 1-salicylalaminoguanidine, may be employed together with an antioxidant in organic substances normally subject to oxidation and containing or in contact with copper and copper-containing metals. They disclose that the 1-(ortho-hydroxy-arylidene)-aminoguanidines act to overcome the catalytic effect of the metals. Such 1-(ortho-hydroxy-arylidene)-aminoguanidines are relatively expensive and it is desirable to produce equivalent or better effects by cheaper materials.

It is an object of this invention to provide petroleum products which have been stabilized against oxidation and deterioration by incorporating therein compounds which are particularly effective both as antioxidants and as copper deactivators. Another object is to provide greases having particularly high resistance to deterioration by oxidation, improved mechanical stability and which will undergo substantially less discoloration during storage and use. A further object is to stabilize petroleum products by means of compounds which are exceptionally effective and yet which are materially less expensive. A still further object is to provide new compositions of matter which are particularly effective as antioxidants for greases and which are cheaper and may be more readily incorporated in greases than prior antioxidant compositions. Further objects are to provide new compositions of matter and to advance the art. Still other objects will appear hereinafter.

The above and other objects may be accomplished in accordance with my invention which comprises incorporating in petroleum products about 0.0001% to about 2% by weight of an equimolecular carboxylic acid salt of a 1-(ortho-hydroxy-arylidene)-aminoguanidine in which the arylidene group is of the benzene series and in which salt the carboxylic acid contains at least 2 carbon atoms and consists of carbon and hydrogen atoms and 1 to 2 carboxyl groups. A particular feature comprises incorporating in a grease, composed substantially wholly of a petroleum oil and a metal soap, about 0.1% to about 2% by weight of a secondary aromatic amine consisting of carbon, hydrogen and 1 to 2 secondary amino nitrogen atoms and in which each of the 2 valences of each nitrogen atom is satisfied by an aromatic radical and about 1% to about 25%, based on the amine, of such an equimolecular carboxylic acid salt of a 1-(ortho-hydroxy-arylidene)-aminoguanidine. My invention also comprises the anti-oxidant compositions composed of about 99% to about 75% of the secondary aromatic amine and about 1% to about 25% of the salt.

I have found that the salts of the 1-(ortho-

hydroxy-arylidene)-aminoguanidines of the character above described are both antioxidants and copper deactivators. They very effectively stabilize petroleum products against oxidation and deterioration in the absence of metal catalysts, such as copper. Also, when the petroleum products are in contact with or contain copper or its catalytically active compounds, such salts are particularly effective to deactivate the copper. I have found further that the combination of secondary aromatic amines and such salts is particularly effective to stabilize greases against oxidation and deterioration during storage and use, both in the presence and in the absence of copper and copper-containing metals. The effect of the combination is greater than the merely cumulative or additive effect of the ingredients. While most of the salts have molecular weights of about 2 to 3 times the molecular weight of the 1-(ortho - hydroxy - arylidene) - aminoguanidine, they are somewhat more effective on the weight basis, and hence have a molecular effectiveness of 2 to 3 times the effectiveness of the free base. Furthermore, the salts cost approximately one-third the cost of the free base. Thus, by my invention, I am able to produce petroleum products of improved stability at nearly one-third the cost. At the same time, the salts inhibit the discoloration of the amines, and hence the antioxidant compositions of amine and salt are more stable toward discoloration.

The petroleum products which are to be stabilized comprise straight-run and cracked gasolines, fuel oils, lubricating oils and lubricating greases. Preferably, the greases are composed substantially wholly of a petroleum oil and a metal soap, such as the soaps of lithium, sodium, potassium, calcium, barium and aluminum. The petroleum oil, employed in producing such greases, will usually be a lubricating oil of the character ordinarily employed in producing greases of this type.

The salts of 1-(ortho-hydroxy-arylidene)-aminoguanidines may be added to the petroleum products as the sole antioxidant or as the sole combined antioxidant and copper deactivator. This has the advantage of obviating the necessity of adding two different agents to the petroleum products—an antioxidant and a copper deactivator. When the petroleum product contains or is in contact with copper or its catalytically active compounds or it is contemplated that it will become contaminated or be brought into contact with copper or its catalytically active compounds, larger amounts of salt will be employed; an amount sufficient to deactivate the copper and an additional amount to thereafter exert the desired antioxidant effect. In some cases, particularly in cracked gasoline and in greases, it will be desired to employ the salt primarily for its copper deactivating effect and to add another antioxidant for the major antioxidant effect. In such latter event, any of the usual antioxidants, known to be effective for the particular petroleum product, may be employed with my salts.

The aromatic amines, which may be employed as antioxidants in greases with the salts, are those ordinarily employed for the stabilization of such greases. Particularly, such aromatic amines are secondary aromatic amines consisting at carbon, hydrogen and 1 to 2 secondary amino nitrogen atoms and in which each of the 2 valences of each nitrogen atom is satisfied by an aromatic radical, that is, the nitrogen is directly bonded to a carbon atom which is a member of

an aromatic ring. Preferably, each aromatic radical contains 1 to 2 benzene rings, that is, is selected from the benzene, naphthalene and biphenyl series. Aromatic amines, which I have found to be particularly desirable in the antioxidant compositions of my invention, are—

Diphenylamine  
Phenyl- $\alpha$ -naphthylamine  
Phenyl- $\beta$ -naphthylamine  
10 Di- $\alpha$ -naphthylamine  
Di- $\beta$ -naphthylamine  
N,N'-diphenyl benzidine  
N,N'-di- $\beta$ -naphthyl-p-phenylenediamine  
N,N'-diphenyl-p-phenylenediamine

15 Still other secondary aromatic amines, which may be employed in such compositions, are—

Ditolylamines  
Phenyl-tolylamines  
Tolyl-naphthylamines  
20 N,N'-ditolyl benzidines  
N,N'-ditolyl-p-phenylenediamines  
N,N'-diphenyl-tolylenediamines  
N,N'-diphenyl-naphthylenediamines  
N,N'-ditolyl-naphthylenediamines

25 The salts, which are to be employed in accordance with my invention, are the equimolecular carboxylic salts of the 1-(ortho-hydroxy-arylidene)-aminoguanidines, that is, the salts formed

30 from equimolecular proportions of the carboxylic acids and the 1-(ortho-hydroxy-arylidene)-aminoguanidines. The 1-(ortho-hydroxy-arylidene)-aminoguanidines, which are employed to produce the salts, are those in which the arylidene group is of the benzene series. The term "arylidene" is employed in its ordinary restricted sense to mean a divalent aromatic radical consisting of carbon and hydrogen. Representative 1-(ortho-hydroxy-arylidene)-aminoguanidines are 1-(salicylalaminoguanidine), 1-(2'-hydroxy-5'-methylbenzal)-aminoguanidine and 1-(2'-hydroxy-5'-ter. - butylbenzal) - aminoguanidine. Of these, 1-salicylalaminoguanidine is preferred.

35 40 45 The 1-(ortho-hydroxy-arylidene)-aminoguanidines may be made by the method disclosed by Wedekind in Ber., 31, 2353 (1898). According to such process, aminoguanidine nitrate is reacted with the ortho-hydroxy-aromatic aldehyde in warm water. Treatment of the resulting mixture with potash solution precipitates the free base.

50 55 60 The acids, which may be employed to produce the salts of my invention, are those carboxylic acids which contain at least 2 carbon atoms and consist of carbon and hydrogen atoms and 1 to 2 carboxyl groups. Preferably, the acids are of the aliphatic series and contain from 6 to 40 carbon atoms and, particularly, those which contain a single carboxyl group. Representative acids, which may be employed to produce satisfactory salts useful in my invention, are—

|                     |                  |
|---------------------|------------------|
| Oleic acid          | Acetic acid      |
| Naphthenic acids    | Linoleic acid    |
| Caproic acids       | Capric acid      |
| Caprylic acid       | Myristic acid    |
| Lauric acid         | Arachidic acid   |
| Palmitic acid       | Behenic acid     |
| Stearic acid        | Cerotic acid     |
| Phenylstearic acid  | Melissic acid    |
| Linoleic acid dimer | Decylenic acid   |
| Sebacic acid        | Undecylenic acid |
| Benzoic acid        | Erucic acid      |

70 75 75 1-salicylalaminoguanidine monoacetate (M. P. 185° C.), 1-salicylaminoguanidine monobenzoate

(M. P. 170° C.) and 1-salicylaminoguanidine monosebacate (M. P. 193° C.) are high melting materials and are only slightly soluble in hydrocarbons, so that it is difficult to properly incorporate them into the petroleum products, and hence such salts are not preferred. On the other hand, the salts of the monocarboxylic aliphatic acids and of linoleic acid dimer melt in the range of about 50° C. to about 98° C. and are fairly soluble in hydrocarbon oils so that they can be readily incorporated into the petroleum products, usually by heating them above their melting points with the oil or grease or a portion thereof. The term "aliphatic" is employed in its broad sense to include acids containing alicyclic rings as well as the acyclic acids. The preferred salts are the 1-salicylaminoguanidine monoleate, 1-salicylaminoguanidine mononaphthenate, and 1-salicylaminoguanidine mono-linoleic acid dimer. The naphthenic acids are usually obtained from crude petroleum or its distillates as mixtures of homologous aliphatic acids containing from 7 to about 20 carbon atoms and a cyclopentane ring carrying alkyl side chains with the carboxyl groups in the side chain and usually on the end of the side chain. The naphthenic acid salts, employed in the examples, were prepared from a mixture of naphthenic acids having an average molecular weight of 242, which corresponds to an average of approximately 15 carbon atoms in each acid molecule. The linoleic acid dimer is a carboxylic acid of the following formula—



The salts of the 1-(ortho-hydroxy-arylidene)-aminoguanidines are advantageously prepared in substantially quantitative yields by mixing substantially equimolecular proportions of the carboxylic acid, an ortho-hydroxy aromatic aldehyde and an inorganic acid salt of the aminoguanidine in an organic solvent with mild heating and then adding water to precipitate the product, which is then filtered and dried. The inorganic acid salts of aminoguanidine, which may be employed in such reaction, are the bicarbonate, the nitrate, the hydrochloride and the phosphate. Since the bicarbonate is a readily available commercial product, it will ordinarily be used. The solvents, which may be used, include aliphatic alcohols of 1 to 4 carbon atoms, such as methyl, ethyl, isopropyl and tertiary butyl alcohols, and liquid aromatic hydrocarbons, such as benzene, toluene and the xylenols. For example, a mixture of 408 grams of aminoguanidine bicarbonate, 373 grams of salicylaldehyde, 840 grams of oleic acid and 300 cc. of methyl alcohol was agitated at 65° C. to 70° C. for 3 hours in a 3 liter glass flask, the reaction mass was added to 3600 cc. of water with stirring, the resulting solid product filtered,

washed with water and air dried, yielding 1426 grams of 1-salicylaminoguanidine monoleate having a melting range of 60° C. to 65° C. This method was followed in preparing the other salts disclosed herein. The methods of preparing the salts are disclosed in more detail in my copending application, Serial No. 94,755, filed May 21, 1949, which claims the preferred salts.

When greases are to be stabilized by a combination of a secondary aromatic amine and a salt, the amount of the amine incorporated in the grease may be from about 0.1% to about 2% by weight, but will usually and preferably be from about 0.25% to about 1%. The salt of the 1-(ortho-hydroxy-arylidene)-aminoguanidine may be employed in the proportion of from about 1% to about 25% by weight, based on the secondary aromatic amine, and preferably from about 5% to about 10%.  
 10 The secondary aromatic amine and the salt of the 1-(ortho-hydroxy-arylidene)-aminoguanidine may be separately added to the grease. However, it will generally be preferred to mix them so as to provide an antioxidant composition composed of the two ingredients in the desired proportion. Such compositions may be made by melting the amine and the salt together, whether the salt appears to dissolve in the amine. The amine and the salt, or the mixtures thereof, will usually be dissolved or dispersed in part of the oil to be employed in manufacturing the grease, but they may be incorporated in the preformed grease by milling or by stirring while heating to melt the inhibitors.

20 In order to more clearly illustrate my invention, preferred modes of carrying the same into effect and advantageous results to be obtained thereby, the following examples are given:

#### EXAMPLE I

40 For the purpose of illustrating the metal deactivating characteristics of these compounds, I have chosen to show the property of salicylaminoguanidine oleate of suppressing the catalytic activity of copper in gasoline. The samples of gasoline, used in the following tests, were completely refined thermal cracked naphtha, untreated with chemical agents such as dyes, antioxidants and anti-knocks. The compounds of the present invention were tested in accordance with 45 A. S. T. M. method D522-46 for the gum stability of gasoline. The results of this test are expressed in terms of "induction period" (in minutes), the period required for oxygen absorption to begin. N-normal butyl-p-aminophenol, abbreviated 50 BAP, has been chosen as a representative gasoline antioxidant. It was added in small quantity to gasoline containing no copper, to the same gasoline containing one part per million of dissolved copper added as the oleate, and to gasoline containing both the dissolved copper and salicylaminoguanidine oleate.

55 The experimental results are given in the following Table I:

Table I

| Concentration     |                  | Deactivator                       | Cone., Wt. Per Cent | Induction Period, Minutes |
|-------------------|------------------|-----------------------------------|---------------------|---------------------------|
| BAP, Wt. Per Cent | Copper, P. P. M. |                                   |                     |                           |
| 0.0               | 0.0              | None.....                         | .....               | 120                       |
| 0.002             | 0.0              | do.....                           | .....               | 423                       |
| 0.002             | 1.0              | do.....                           | .....               | 170                       |
| 0.002             | 1.0              | Salicylaminoguanidine oleate..... | 0.0005              | 391                       |
| 0.002             | 1.0              | do.....                           | 0.001               | 430                       |

7 It will be observed that the catalytic effect of copper is counteracted by this compound.

EXAMPLE II

To illustrate the utility of the compounds of this invention as antioxidants for gasoline, they were evaluated in cracked gasoline which had been thoroughly refined to remove metals. The antioxidant characteristics were compared with 2,6-ditertiarybutyl-4-methylphenol which is a well established commercial gasoline antioxidant.

The various products shown below were added at 0.005% by weight to the gasoline and the induction periods were then determined by the method described in Example I. The weight effectiveness of 2,6-ditertiary-4-methylphenol, which at 0.005 wt. per cent increased the induction period from 185 to 243 minutes, was arbitrarily assigned the molar efficiency of 100.

The experimental results are given in the following Table II:

Table II

| Antioxidant                                        | Induction Period, Minutes | Per Cent Efficiency |             |
|----------------------------------------------------|---------------------------|---------------------|-------------|
|                                                    |                           | Wt. Basis           | Molar Basis |
| None                                               | 185                       |                     |             |
| 2,6-ditertiarybutyl-4-methylphenol                 | 243                       | 100                 |             |
| 1-Salicylalaminoguanidine base                     | 203                       | 186                 | 100         |
| 1-Salicylalaminoguanidine mononaphthenate          | 248                       | 108                 | 139         |
| 1-Salicylalaminoguanidine monolaurate              | 271                       | 148                 | 169         |
| 1-Salicylalaminoguanidine monocaproate             | 268                       | 143                 | 136         |
| 1-Salicylalaminoguanidine monolinolenic acid dimer | 256                       | 122                 | 174         |
| 1-Salicylalaminoguanidine monoleate                | 255                       | 120                 | 167         |

It will be observed that the compounds of this invention are effective gasoline antioxidants and

8 lar test used is commonly referred to as the "Accelerated Norma-Hoffman Stability Test" and is described in the proceedings of the American Society for Testing Materials, volume 38, part II, 5 1938, in an article entitled, "Some applications of an accelerated test for determining the chemical stability of lubricating greases." In this test a weighed sample of the grease to be tested is 10 charged into a glass container, with or without brass catalyst, and the container is placed in a suitable bomb and subjected to a pressure of 110 pounds of oxygen at 210° to 212° F. for a certain number of hours or until the pressure has dropped 15 a certain number of pounds.

In these experiments, all of the samples were run in the presence of brass. Included in the products tested were samples treated with phenyl- 20 α-naphthylamine, which is a conventional grease stabilizer having wide commercial application,

and with salicylalaminoguanidine base, respectively. The results are shown in Table III:

Table III

| Stabilizers                                  | Norma-Hoffman Stability Test—Hours to 25 lbs./sq. in. pressure drop |
|----------------------------------------------|---------------------------------------------------------------------|
| None (unstabilized)                          | 14                                                                  |
| 0.5% phenyl-α-naphthylamine                  | 55                                                                  |
| 0.5% 1-salicylalaminoguanidine base          | 104                                                                 |
| 0.5% 1-salicylalaminoguanidine monocaproate  | 150                                                                 |
| 0.5% 1-salicylalaminoguanidine monocaprylate | 144                                                                 |
| 0.5% 1-salicylalaminoguanidine monolaurate   | 123                                                                 |
| 0.5% 1-salicylalaminoguanidine monobenzoate  | 164                                                                 |
| 0.5% 1-salicylalaminoguanidine monobebacate  | 158                                                                 |
| 0.5% 1-salicylalaminoguanidine monopalmitate | 126                                                                 |

that their molar effectiveness is much higher than the salicylalaminoguanidine base.

EXAMPLE III

As another example of the usefulness of the compounds of this invention, samples of a commercial unstabilized calcium soap grease were treated with 0.5% by weight of several different organic acid salts of salicylalaminoguanidine. The products were incorporated into the grease samples by working the grease and the salt together on a porcelain plate with a spatula for one hour.

The grease samples were subjected to an accelerated oxidation stability test. The particu-

EXAMPLE IV

60 Samples of a commercial unstabilized calcium soap grease were treated with 0.45% by weight of various secondary aromatic amides together with 0.05% of 1-salicylalaminoguanidine monoleate (A), making 0.5% by weight of total stabilizers based on the grease. Samples of the same grease 65 were treated with 0.5% by weight of the amines alone and still another sample was treated with 0.5% of 1-salicylalaminoguanidine monoleate (A) alone.

The stabilizers were incorporated into the commercial samples and the samples were tested in the same way as in Example III.

In this particular set of experiments, the greases were all run in the presence of brass disks to 25 pounds' pressure drop. The results of the 75 tests are as follows:

Table IV

| No. | Stabilizers added to the grease                                 | Hours to 25 Pounds'<br>Pressure Drop |
|-----|-----------------------------------------------------------------|--------------------------------------|
| 1   | None                                                            | 14                                   |
| 2   | 0.5% 1-salicylalaminoguanidine monoleate (A)                    | 110                                  |
| 3   | 0.5% phenyl- $\alpha$ -naphthylamine                            | 55                                   |
| 4   | 0.45% phenyl- $\alpha$ -naphthylamine + 0.05% (A)               | 94                                   |
| 5   | 0.5% phenyl- $\beta$ -naphthylamine                             | 40                                   |
| 6   | 0.45% phenyl- $\beta$ -naphthylamine + 0.05% (A)                | 56                                   |
| 7   | 0.5% di- $\alpha$ -naphthylamine                                | 54                                   |
| 8   | 0.45% di- $\alpha$ -naphthylamine + 0.05% (A)                   | 78                                   |
| 9   | 0.5% N,N'-diphenyl benzidine                                    | 42                                   |
| 10  | 0.45% N,N'-diphenyl benzidine + 0.05% (A)                       | 62                                   |
| 11  | 0.5% N,N'-di- $\beta$ -naphthyl-p-phenylenediamine              | 68                                   |
| 12  | 0.45% N,N'-di- $\beta$ -naphthyl-p-phenylenediamine + 0.05% (A) | 104                                  |
| 13  | 0.05% N,N'-diphenyl-p-phenylenediamine                          | 84                                   |
| 14  | 0.45% N,N'-diphenyl-p-phenylenediamine + 0.05% (A)              | 96                                   |
| 15  | 0.5% diphenylamine                                              | 106                                  |
| 16  | 0.45% diphenylamine + 0.05% (A)                                 | 142                                  |

It will be noted that, in every case, the effect of the combination of stabilizers is materially greater than the mere cumulative effect of the components of the combination.

#### EXAMPLE V

Samples of a commercial, unstabilized calcium soap grease were treated with 0.45% diphenylamine together with 0.05% by weight, based on the grease (10% by weight based on the diphenylamine), of various equimolecular carboxylic acid salts of 1-salicylalaminoguanidine. A sample of the same grease was treated with 0.5% by weight of diphenylamine and still other samples were treated with 0.5% by weight of some of the salts of 1-salicylalaminoguanidine alone. The various stabilizers were homogeneously mixed with the grease as described in Example III.

The grease samples were subjected to the Norma-Hoffman accelerated oxidation stability test as described in Example III. In this set of experiments, the grease samples were all run in the presence of brass disks to 25 pounds' pressure drop. The results of the test are as follows:

Table V

| No. | Stabilizers added                                                             | Hours to 25 Pounds'<br>Pressure Drop |
|-----|-------------------------------------------------------------------------------|--------------------------------------|
| 1   | None                                                                          | 14                                   |
| 2   | 0.5% diphenylamine                                                            | 106                                  |
| 3   | 0.45% diphenylamine + 0.05% 1-salicylalaminoguanidine monoacetate             | 130                                  |
| 4   | 0.45% diphenylamine + 0.05% 1-salicylalaminoguanidine monocaprylate           | 142                                  |
| 5   | 0.45% diphenylamine + 0.05% 1-salicylalaminoguanidine monocaprate             | 132                                  |
| 6   | 0.5% 1-salicylalaminoguanidine monolaurate                                    | 123                                  |
| 7   | 0.45% diphenylamine + 0.05% 1-salicylalaminoguanidine monolaurate             | 142                                  |
| 8   | 0.5% 1-salicylalaminoguanidine monophenylstearate                             | 53                                   |
| 9   | 0.45% diphenylamine + 0.05% 1-salicylalaminoguanidine monophenylstearate      | 130                                  |
| 10  | 0.45% diphenylamine + 0.05% 1-salicylalaminoguanidine monolinoleic acid dimer | 142                                  |
| 11  | 0.45% diphenylamine + 0.05% 1-salicylalaminoguanidine monobenzoate            | 118                                  |
| 12  | 0.45% diphenylamine + 0.05% 1-salicylalaminoguanidine monosebacate            | 125                                  |
| 13  | 0.5% 1-salicylalaminoguanidine mononaphthalenes                               | 64                                   |
| 14  | 0.45% diphenylamine + 0.05% 1-salicylalaminoguanidine mononaphthalenes        | 146                                  |
| 15  | 0.45% diphenylamine + 0.05% 1-salicylalaminoguanidine monopalmitate           | 126                                  |
| 16  | 0.45% diphenylamine + 0.05% 1-salicylalaminoguanidine monostearate            | 130                                  |

#### EXAMPLE VI

Unstabilized commercial greases of several different metal soaps were treated with varying amounts of a stabilizer composition consisting of a mixture of 90% diphenylamine and 10% 1-salicylalaminoguanidine monoleate. The stabilizer composition was added to the grease sample as described in Example III.

The treated grease samples and control samples

70 1-salicylalaminoguanidine monoleate and with 0.5% by weight of mixtures of diphenylamine with 1%, 5%, 10%, 15%, 20% and 25% of 1-salicylalaminoguanidine monoleate.

The samples were prepared for testing by thoroughly mixing the stabilizers with the grease as described in Example III. The grease samples were tested by the Norma-Hoffman accelerated oxidation method which is described in Example

20 of the same greases were subjected to the Norma-Hoffman accelerated oxidation stability test as described in Example III. These tests were made in the absence of added metal catalysts. The results of the tests are as follows:

Table VI

| 25 | Grease                     | Concentration<br>Wt. Per Cent<br>of Stabilizer | Pounds'<br>Pressure<br>Drop | Hours<br>Run |
|----|----------------------------|------------------------------------------------|-----------------------------|--------------|
| 30 | Lithium soap grease        | 0.0                                            | 25                          | 162          |
|    |                            | 0.1                                            | 8                           | 360          |
| 35 | Calcium soap grease        | 0.25                                           | 6                           | 360          |
|    |                            | 0.0                                            | 25                          | 70           |
| 35 | Sodium soap grease         | 0.25                                           | 22                          | 360          |
|    |                            | 0.0                                            | 25                          | 260          |
| 35 | Sodium-calcium soap grease | 1.0                                            | 18                          | 360          |
|    |                            | 0.0                                            | 25                          | 33           |
| 35 | Sodium-calcium soap grease | 0.5                                            | 25                          | 360          |
|    |                            | 1.0                                            | 24                          | 360          |

#### EXAMPLE VII

Samples of a commercial, unstabilized calcium soap grease were treated with 0.5% by weight 40 of diphenylamine, with 0.5% by weight of

III. In this set of experiments, the grease samples were all run in the presence of brass disks, which served as a catalyst, to 25 pounds' pressure drop. The effect of various proportionate amounts of 1-salicylaminoguanidine monoleate (abbreviated to SAG-monoleate) together with diphenylamine (abbreviated to DPA) are given in the following Table VII:

Table VII

| No. | Stabilizers added                             | Hours to 25 Pounds' Pressure Drop |
|-----|-----------------------------------------------|-----------------------------------|
| 1.  | None (unstabilized)                           |                                   |
| 2.  | 0.5% DPA                                      | 14                                |
| 3.  | 0.5% mixture of 99% DPA and 1% SAG-monoleate  | 106                               |
| 4.  | 0.5% mixture of 95% DPA and 5% SAG-monoleate  | 126                               |
| 5.  | 0.5% mixture of 90% DPA and 10% SAG-monoleate | 148                               |
| 6.  | 0.5% mixture of 85% DPA and 15% SAG-monoleate | 170                               |
| 7.  | 0.5% mixture of 80% DPA and 20% SAG-monoleate | 142                               |
| 8.  | 0.5% mixture of 75% DPA and 25% SAG-monoleate | 138                               |
| 9.  | 0.5% SAG-monoleate                            | 118                               |
|     |                                               | 100                               |

This example particularly illustrates that the combination of stabilizers unexpectedly produces results considerably superior to the mere additive effects of the individual components. Since diphenylamine gave a value of 106 and the 1-salicylaminoguanidine monoleate gave a value of 100, it would be expected that the values of Nos. 3 to 8 would be between 106 and 100, such values decreasing as increasing amounts of the diphenylamine were replaced by 1-salicylaminoguanidine monoleate.

## EXAMPLE VIII

Samples of commercial unstabilized greases, a calcium soap grease and a sodium soap grease, were treated with diphenylamine, mixtures of diphenylamine and 1-salicylaminoguanidine base (abbreviated to SAG), and mixtures of diphenylamine and 1-salicylaminoguanidine monoleate (abbreviated to SAG-oleate) in the manner described in Example III. These samples were subjected to the Norma-Hoffman Stability Test as described in Example III, tests being run both with and without the brass catalyst. The proportions and results are shown in Table VIII:

Table VIII

| No. | Grease Composition                      | No Catalyst |                      | Brass |                      |
|-----|-----------------------------------------|-------------|----------------------|-------|----------------------|
|     |                                         | Hrs.        | Pounds Pressure Drop | Hrs.  | Pounds Pressure Drop |
| 1.  | Grease (calcium soap) (A)               | 70          | 25                   | 14    | 25                   |
| 2.  | (A)+0.5% diphenylamine                  | 430         | 25                   | 139   | 25                   |
| 3.  | (A)+4.5% diphenylamine+0.05% SAG (base) | 500         | 21                   | 162   | 25                   |
| 4.  | (A)+4.5% diphenylamine+0.05% SAG-oleate | 500         | 20                   | 170   | 25                   |
| 5.  | Grease (sodium soap) (B)                | 33          | 25                   | 12    | 25                   |
| 6.  | (B)+0.5% diphenylamine                  | 336         | 25                   | 112   | 25                   |
| 7.  | (B)+4.5% diphenylamine+0.05% SAG (base) | 406         | 25                   | 129   | 25                   |
| 8.  | (B)+4.5% diphenylamine+0.05% SAG-oleate | 486         | 25                   | 130   | 25                   |

From the above results, it will be seen that the 1-salicylaminoguanidine monoleate (the salt) is somewhat more effective than the 1-salicylaminoguanidine (the base) on the weight basis. However, the salt (mol. wt.=459.6) has a molecular weight about 2.6 times that of the base (mol. wt.=177.1) and hence the mole ratios of base and salt employed were about 2.6 to 1. Thus, it is apparent that 1 mole of the salt is more than 2.6 times as effective as 1 mole of the base, both in the presence and in the absence of a brass catalyst.

Moreover, the fatty acid and napthenic acid salts of salicylaminoguanidine can be prepared

at a cost of about 37% of the cost of the base. Accordingly, my invention makes it possible to obtain improved results at approximately 1/3 the cost.

It will be understood that the preceding examples have been given for illustrative purposes solely and that my invention is not limited to the specific embodiments disclosed therein. It

will be readily apparent to those skilled in the art that many variations and modifications can be made within the limits hereinbefore set forth without departing from the spirit or scope of my invention.

It will be apparent that, by my invention, I am able to produce petroleum products of substantially improved stability toward deterioration and oxidation and at a substantial reduction in cost. The preferred salts of the 1-(ortho-hydroxy-arylidene)-aminoguanidines of my invention have lower melting points than the free base and are more soluble in hydrocarbons so that they may be more readily incorporated in petroleum products and, particularly, in oils and greases. It is also apparent that I am able to provide new, more stable, more effective and less expensive antioxidant compositions which may be readily and easily incorporated in oils and greases. Therefore, it will be apparent that my invention constitutes a valuable advance and contribution to the art.

I claim:

1. A petroleum product having incorporated therein about 0.0001% to about 2% of an equi-

molecular carboxylic acid salt of a 1-(ortho-hydroxy-arylidene)-aminoguanidine in which the arylidene group is of the benzene series and in which salt the carboxylic acid contains at least 2 carbon atoms and consists of carbon and hydrogen atoms and 1 to 2 carboxyl groups.

2. A petroleum product having incorporated therein about 0.0001% to about 2% of an equimolecular carboxylic acid salt of a 1-(ortho-hydroxy-arylidene)-aminoguanidine in which the arylidene group is of the benzene series and in which salt the carboxylic acid is of the aliphatic series, contains 6 to 40 carbon atoms and consists of carbon and hydrogen atoms and 1 to 2

carboxyl groups; said salt having a melting point in the range of about 50° C. to about 98° C.

3. A petroleum product having incorporated therein about 0.0001% to about 2% of an equimolecular carboxylic acid salt of a 1-(ortho-hydroxy-arylidene)-aminoguanidine in which the arylidene group is of the benzene series and in which salt the carboxylic acid is of the aliphatic series, contains 6 to 40 carbon atoms and consists of carbon and hydrogen atoms and 1 carboxyl group; said salt having a melting point in the range of about 50° C. to about 98° C.

4. A petroleum product having incorporated therein about 0.0001% to about 2% of a 1-(ortho-hydroxy-arylidene)-aminoguanidine monoleate in which the arylidene group is of the benzene series.

5. A petroleum product having incorporated therein about 0.0001% to about 2% of a 1-(ortho-hydroxy-arylidene)-aminoguanidine mononaphthenate in which the arylidene group is of the benzene series.

6. A grease, composed substantially wholly of a petroleum oil and a metal soap, having incorporated therein about 0.001% to about 2% of an equimolecular carboxylic acid salt of a 1-(ortho-hydroxy-arylidene)-aminoguanidine in which the arylidene group is of the benzene series and in which salt the carboxylic acid contains at least 2 carbon atoms and consists of carbon and hydrogen atoms and 1 to 2 carboxyl groups.

7. A grease, composed substantially wholly of a petroleum oil and a metal soap, having incorporated therein about 0.001% to about 2% of an equimolecular carboxylic acid salt of a 1-(ortho-hydroxy-arylidene)-aminoguanidine in which the arylidene group is of the benzene series and in which salt the carboxylic acid is of the aliphatic series, contains 6 to 40 carbon atoms and consists of carbon and hydrogen atoms and 1 to 2 carboxyl groups; said salt having a melting point in the range of about 50° C. to about 98° C.

8. A grease, composed substantially wholly of a petroleum oil and a metal soap, having incorporated therein about 0.001% to about 2% of an equimolecular carboxylic acid salt of a 1-(ortho-hydroxy-arylidene)-aminoguanidine in which the arylidene group is of the benzene series and in which salt the carboxylic acid is of the aliphatic series, contains 6 to 40 carbon atoms and consists of carbon and hydrogen atoms and 1 carboxyl group; said salt having a melting point in the range of about 50° C to about 98° C.

9. A grease, composed substantially wholly of a petroleum oil and a metal soap, having incorporated therein about 0.1% to about 2% of a secondary aromatic amine consisting of carbon, hydrogen and 1 to 2 secondary amino nitrogen atoms and in which each of the two valences of each nitrogen atom is satisfied by an aromatic radical containing 1 to 2 benzene rings; and about 1% to about 25%, based on the amine, of an equimolecular carboxylic acid salt of a 1-(ortho-hydroxy-arylidene)-aminoguanidine in which the arylidene group is of the benzene series and in which salt the carboxylic acid contains at least 2 carbon atoms and consists of carbon and hydrogen atoms and 1 to 2 carboxyl groups.

10. A grease, composed substantially wholly of a petroleum oil and a metal soap, having incorporated therein about 0.1% to about 2% of a secondary aromatic amine consisting of carbon, hydrogen and 1 to 2 secondary amino nitrogen atoms and in which each of the two valences of each nitrogen atom is satisfied by an aromatic

radical containing 1 to 2 benzene rings; and about 1% to about 25%, based on the amine, of an equimolecular carboxylic acid salt of 1-salicylaminoguanidine in which the carboxylic acid contains at least 2 carbon atoms and consists of carbon and hydrogen atoms and 1 to 2 carboxyl groups.

11. A grease, composed substantially wholly of a petroleum oil and a metal soap, having incorporated therein about 0.1% to about 2% of a secondary aromatic amine consisting of carbon, hydrogen and 1 to 2 secondary amino nitrogen atoms and in which each of the two valences of each nitrogen atom is satisfied by an aromatic radical containing 1 to 2 benzene rings; and about 1% to about 25%, based on the amine, of an equimolecular carboxylic acid salt of 1-salicylaminoguanidine in which the carboxylic acid is of the aliphatic series, contains 6 to 40 carbon atoms and consists of carbon and hydrogen atoms and 1 to 2 carboxyl groups; said salt having a melting point in the range of about 50° C. to about 98° C.

12. Gasoline having incorporated therein about 0.0001% to about 0.01% of an equimolecular carboxylic acid salt of a 1-(ortho-hydroxy-arylidene)-aminoguanidine in which the arylidene group is of the benzene series and in which salt the carboxylic acid contains at least 2 carbon atoms and consists of carbon and hydrogen atoms and 1 to 2 carboxyl groups.

13. Gasoline having incorporated therein about 0.0001% to about 0.01% of an equimolecular carboxylic acid salt of a 1-(ortho-hydroxy-arylidene)-aminoguanidine in which the arylidene group is of the benzene series and in which salt the carboxylic acid is of the aliphatic series, contains 6 to 40 carbon atoms and consists of carbon and hydrogen atoms and 1 to 2 carboxyl groups; said salt having a melting point in the range of about 50° C. to about 98° C.

14. A composition composed of about 99% to about 75% of a secondary aromatic amine consisting of carbon, hydrogen and 1 to 2 secondary amino nitrogen atoms and in which each of the two valences of each nitrogen atom is satisfied by an aromatic radical; and about 1% to about 25% of an equimolecular carboxylic acid salt of a 1-(ortho-hydroxy-arylidene)-aminoguanidine in which the arylidene group is of the benzene series and in which salt the carboxylic acid contains at least 2 carbon atoms and consists of carbon and hydrogen atoms and 1 to 2 carboxyl groups.

15. A composition composed of about 99% to about 75% of a secondary aromatic amine consisting of carbon, hydrogen and 1 to 2 secondary amino nitrogen atoms and in which each of the two valences of each nitrogen atom is satisfied by an aromatic radical; and about 1% to about 25% of an equimolecular carboxylic acid salt of a 1-(ortho-hydroxy-arylidene)-aminoguanidine in which the arylidene group is of the benzene series and in which salt the carboxylic acid is of the aliphatic series, contains 6 to 40 carbon atoms and consists of carbon and hydrogen atoms and 1 carboxyl group; said salt having a melting point in the range of about 50° C. to about 98° C.

16. A composition composed of about 99% to about 75% of a secondary aromatic amine consisting of carbon, hydrogen and 1 to 2 secondary amino nitrogen atoms and in which each of the two valences of each nitrogen atom is satisfied by an aromatic radical containing 1 to 2 benzene rings; and about 1% to about 25% of an equimolecular carboxylic acid salt of 1-salicyl-

alaminoguanidine in which the carboxylic acid contains at least 2 carbon atoms and consists of carbon and hydrogen atoms and 1 to 2 carboxyl groups.

17. A composition composed of about 99% to about 75% of a secondary aromatic amine consisting of carbon, hydrogen and 1 to 2 secondary amino nitrogen atoms and in which each of the two valences of each nitrogen atom is satisfied by an aromatic radical containing 1 to 2 benzene rings; and about 1% to about 25% of an equimolecular carboxylic acid salt of 1-salicyl-alaminoguanidine in which the carboxylic acid is of the aliphatic series, contains 6 to 40 carbon atoms and consists of carbon and hydrogen atoms and 1 to 2 carboxyl groups; said salt having a melting point in the range of about 50° C. to about 98° C.

18. A composition composed of about 99% to about 75% of a secondary aromatic amine consisting of carbon, hydrogen and 1 to 2 secondary amino nitrogen atoms and in which each of the two valences of each nitrogen atom is satisfied by an aromatic radical containing 1 to 2 benzene rings; and about 1% to about 25% of an equimolecular carboxylic acid salt of 1-salicyl-alaminoguanidine in which the carboxylic acid is of the aliphatic series, contains 6 to 40 carbon atoms and consists of carbon and hydrogen atoms and 1 carboxyl group; said salt having a melting point in the range of about 50° C. to about 98° C.

19. A composition composed of about 99% to about 75% of a secondary aromatic amine con-

sisting of carbon, hydrogen and 1 to 2 secondary amino nitrogen atoms and in which each of the two valences of each nitrogen atom is satisfied by an aromatic radical containing 1 to 2 benzene rings; and about 1% to about 25% of 1-salicyl-alaminoguanidine monoleate.

20. A composition composed of about 99% to about 75% of a secondary aromatic amine consisting of carbon, hydrogen and 1 to 2 secondary amino nitrogen atoms and in which each of the two valences of each nitrogen atom is satisfied by an aromatic radical containing 1 to 2 benzene rings; and about 1% to about 25% of 1-salicyl-alaminoguanidine mononaphthenate.

CHARLES B. BISWELL.

#### REFERENCES CITED

The following references are of record in the file of this patent:

#### UNITED STATES PATENTS

| Number    | Name             | Date          |
|-----------|------------------|---------------|
| 2,221,207 | Sibley           | Nov. 12, 1940 |
| 2,243,485 | Musselman        | May 27, 1941  |
| 2,275,264 | Musselman et al. | Mar. 3, 1942  |
| 2,282,513 | Downing et al.   | May 12, 1942  |
| 2,323,948 | Von Bramer       | July 13, 1943 |
| 2,353,690 | Clarkson et al.  | July 18, 1944 |
| 2,361,339 | White et al.     | Oct. 24, 1944 |
| 2,469,745 | Robertson        | May 10, 1949  |
| 2,480,449 | Cocroft et al.   | Aug. 30, 1949 |
| 2,503,969 | Rudel et al.     | Apr. 11, 1950 |
| 2,515,133 | Morway           | July 11, 1950 |